

Jan. 18, 1966

J. J. RAUSCH ET AL

3,230,080

COBALT BASE ALLOYS CONTAINING TITANIUM

Filed Sept. 24, 1963



TENSILE PROPERTIES OF COBALT ALLOYED  
WITH TITANIUM

INVENTORS

JOHN J. RAUSCH  
JOSEPH B. Mc ANDREW

BY

*Claude Tunkhouse*  
*Kenneths Prestorf* ATTORNEY  
AGENT

## 1

3,230,080  
COBALT BASE ALLOYS CONTAINING  
TITANIUM

John J. Rausch, Evanston, Ill., and Joseph B. McAndrew, Pittsburgh, Pa., assignors, by mesne assignments, to the United States of America as represented by the Secretary of the Navy

Filed Sept. 24, 1963, Ser. No. 311,266  
2 Claims. (Cl. 75—170)

The present invention relates to improved cobalt alloys and to methods of making the same. More particularly, the present invention relates to cobalt base alloys having improved physical and metallurgical properties.

The present commercial cobalt alloys do not provide the strength capabilities under extreme conditions of high temperature and in a highly oxidative environment as required in the neoteric nuclear, missile and space technologies. It is necessary under these conditions to provide an alloy having high temperature oxidation resistance, high temperature strength and workability.

Accordingly, features and objects of this invention include the provision of new composition with optimum strength and acceptable oxidation resistance at high temperatures.

Another object of the present invention is to provide an alloy of cobalt that is strong and ductile, while retaining sufficient forgeability to be usefully workable.

A further object of the present invention is to provide a novel, wrought cobalt base alloy that is superior in properties to those presently used for high temperature application.

Other objects and many of the attendant advantages of this invention will be readily appreciated as the same becomes better understood by reference to the following detailed description when considered in connection with the accompanying tables and graphs wherein the figure is a graphical presentation of the effect of titanium addition on the properties of the wrought cobalt base.

The alloy which satisfies the objects of the present invention in its broadest aspect consists essentially of from 1 to 10 weight percent titanium with the balance essentially all cobalt. The significance of titanium as a cobalt strengthener may be seen by referring to the accompanying graph. The ductility of the alloy, which may also be seen in the graph, was considered to be an important indicator of the fabricability of the material.

Although the foregoing alloys satisfy all of the objects set forth above, it was determined that by the addition of a third element to the binary alloy composition, elevated temperature strength, forgeability and oxidation resistance could be improved. The effect of ternary additions on the 1700° F. tensile properties of the base composition cobalt-10 weight percent titanium is shown in Table I. The test alloys were aged 24 hours at 1700° F.

Table I

| Alloy       | YS (p.s.i.) | RA (percent) |
|-------------|-------------|--------------|
| Co-10Ti-1Cb | 60,000      | 15           |
| Co-10Ti-3Ta | 58,000      | 27           |

Ternary alloys based on cobalt-ten weight percent titanium were generally not forgeable. The additions of 2% silicon, 1% columbium and 3% tantalum, however, produced alloys that could be readily fabricated into bar stock. Of these, the latter two had desirable high-temperature strength properties as shown in Table I.

## 2

In the preparation of the cobalt base alloys, two grades of cobalt were employed, typical analyses of which are given below:

Table II

| Elements  | Rondell Cobalt (percent) | Electrolytic Cobalt (percent) |
|-----------|--------------------------|-------------------------------|
| Cobalt    | 99.29                    | 99.6                          |
| Nickel    | 0.28                     | 0.20                          |
| Iron      | 0.03                     | 0.05                          |
| Copper    | nil                      | 0.01                          |
| Carbon    | 0.04                     | 0.05                          |
| Calcium   | 0.02                     | —                             |
| Manganese | 0.03                     | trace                         |
| Silicon   | 0.04                     | 0.01                          |
| Sulphur   | 0.01                     | 0.01                          |

Electrolytic cobalt was found to be the more favorable base metal since this material is forgeable without the use of modifiers or special melting techniques. The alloys of the instant invention and the elements therein were, in general, of equivalent or better purity than the electrolytic cobalt. The tantalum and columbium used were in the form of high purity sheet.

Alloys were prepared as 250 gram, pancake shaped ingots approximately  $\frac{1}{2}$ " x 3" in diameter. These were arc-melted using a water-cooled tungsten-tipped electrode and a water-cooled, copper crucible in an argon atmosphere. The ingots were then hammer-forged to  $\frac{1}{2}$ " in diameter rods from which test specimens were prepared.

Tensile tests were performed at room temperature and at 1700° F. at a strain rate of approximately 0.12 in./in./minute. Before testing, all specimens were sealed in evacuated bulbs, treated at 1700° F. for 24 hours and air-cooled.

In the present invention and dependent claims, the phrase "up to" shall be construed to include zero as the lower limit of the percentage range of optional elements recited.

It will be apparent that new and useful alloys having desirable characteristics and properties have been disclosed. It is therefore desired to further describe the invention as set forth in the appended claims.

What is claimed is:

1. A forgeable high-strength alloy consisting essentially of about 1 to 10 weight percent titanium, about 1 weight percent columbium, the balance being cobalt.
2. A forgeable alloy having high-strength at elevated temperatures consisting essentially of about 1 to 10 weight percent titanium, about 3 weight percent tantalum, the balance being cobalt.

## References Cited by the Examiner

## UNITED STATES PATENTS

2,983,602 5/1961; Levinson et al. — 75—170

## OTHER REFERENCES

60 Hansen: Constitution of Binary Alloys, 2nd edition, published by McGraw-Hill Book Company, New York, N.Y., 1958, pages 511-514.

The Journal of the Institute of Metals, volume XLIV, No. 2, 1930, page 492.

65 DAVID L. RECK, Primary Examiner.

WINSTON A. DOUGLAS, Examiner.

C. M. SCHUTZMAN, R. O. DEAN, Assistant Examiners.